

## UNITED STATES PATENT OFFICE

2,427,242

## TEXTILE SOFTENING COMPOSITION

Emil A. Vitalis, East Port Chester, and John E. Lynn, Old Greenwich, Conn., assignors to American Cyanamid Company, New York, N. Y., a corporation of Maine

No Drawing. Application May 14, 1945,  
Serial No. 593,758

19 Claims. (CL 252—8.75)

1

This invention relates to the softening of textiles such as wool, cotton, rayon, and nylon cloth, and is directed more particularly to the provision of softening compositions having improved permanency and softening properties. The invention includes the novel softening compositions themselves, their methods of preparation, and improved methods for the finishing of textile fabrics, threads, and fibers with the aid of these softening compositions as will hereinafter be described.

Although a wide variety of softening materials of the class of oils, waxes and the like have been proposed for improving the softness of hand of textiles, there is still a demand for softeners of improved permanency and laundry-resistance. Many of the compositions now sold on the market will produce a temporary softening effect, but the textiles soon become limp and raggy after they have been laundered several times. This is true even of the so-called cationic softeners, which are supposed to combine permanently with textiles through the action of an opposite electrical charge, but many of which lose softening power almost completely by repeated launderings.

It is a principal object of the present invention to provide textile softening compositions which can be used either alone or in conjunction with other finishing agents to produce finished textiles having a soft and elastic hand which is not removed by repeated launderings. A still further object is the provision of textile finishing compositions in the form of water-dispersible pastes which are stable upon storage. Other objects of the invention will appear from the following description of preferred embodiments thereof.

In the copending application of J. T. Thurston and W. N. Oldham, Serial No. 542,246, filed June 26, 1944, there is described a new class of compounds obtained by condensing the reaction products of carbon dioxide and higher primary aliphatic amines containing 12 or more carbon atoms with aqueous cyanamide solutions. The products of this reaction contain guanidinium salts of N-aliphatic substituted carbamic acids in which both the guanidine and the carbamic acid are substituted by long aliphatic radicals of the amine used. In some of the examples of this application the reaction of the amine salts with the cyanamide solution is not carried to completion and the product therefore contains higher aliphatic amine salts of N-aliphatic substituted carbamic acids in addition to the aliphatic substituted guanidinium N-aliphatic carbamates. Both types of reaction products are converted

2

into a water-soluble condition by further condensation with alkylene oxides of 2-4 carbon atoms such as ethylene, propylene or butylene oxide, and in this condition they are shown to be good cationic softening agents for textiles.

Our present invention is based on the discovery that the addition of anion-active surface-active agents having single long aliphatic chain of 12 or more and preferably 16-18 carbon atoms to certain of the compositions described in the Thurston et al. application will result in textile finishing compositions of greatly improved permanency and laundry-resistance. In its broader aspects, therefore, our invention consists in the provision of a mixture containing a major quantity of the reaction product of an alkylene oxide of 2-4 carbon atoms with mixed N-aliphatic carbamic acid salts of aliphatic-substituted guanidines and amines in which all the aliphatic radicals contain 12 or more carbon atoms together with a smaller quantity of an anionic surface-active agent containing a single long aliphatic radical of 12 or more carbon atoms.

We have found that the addition of an aqueous solution of an anionic surface-active agent containing a single long aliphatic radical to aqueous solutions of the above-described alkylene oxide condensation products will result in the formation of dispersions which possess good softening action on cotton, rayon, wool, nylon and other threads, filaments, and fabrics but which can be converted to a water-insoluble and laundry-resistant condition by heating textiles impregnated therewith for short periods of time. These mixtures may be applied to the textiles alone or in conjunction with small quantities on the order of 0.1-4% of water-soluble polyvalent metal salts such as aluminum sulfate, zinc sulfate, zirconium acetate and the like. They may be applied as such or in conjunction with starch or resin finishes. In all cases, however, it will be found that a marked improvement in the permanency of the finish is obtained, as compared with the laundry-resistance of cationic softeners to which no anionic wetting agent of the type described has been added.

Any primary aliphatic amine of 12-18 or more carbon atoms may be used in preparing the compositions of our invention. We prefer the aliphatic amines in which the aliphatic radical contains 16-18 or more carbon atoms, since finishes of better permanency are obtained therefrom. The aliphatic radical may be either saturated or unsaturated, for we have found that even a relatively high degree of unsaturation does not cause

rancidity or discoloration after the finish has been applied to fabrics. This is probably due to the stabilizing or antioxidant properties of the guanidine radical. This fact permits us to employ carbamates prepared from mixtures of higher aliphatic amines, such as are now available on the market at low cost and in large quantities. One such mixture which we have used with advantage contains about 20-30% of hexadecyl amine and about 70-80% of a mixture of saturated and unsaturated amines of 18 carbon atoms.

We have found that optimum results are obtained when only a part of the higher aliphatic amines are converted into guanidine salts. Preferably the reaction with cyanamide is so controlled that about 50-70% of the amines are converted into guanidinium carbamates of the formula



in which R is a saturated or unsaturated aliphatic radical of 12 or more carbon atoms corresponding to the amine used, while the remainder is present in the form of an amine salt of an N-substituted carbamic acid of the formula



in which R is as defined above. Under these conditions the reaction product contains about 15-25 mol percent of unreacted amine, about 50 mol percent of N-aliphatic-substituted carbamic acid and about 25-35 mol percent of aliphatic-substituted guanidine, based on the total quantity of amines used. Cationic softeners of optimum properties for use in the compositions of our invention are obtained when reaction products having these percentage compositions are condensed with 2-10 mols of alkylene oxides.

The quantities of alkylene oxide condensed with the mixture of carbamic acid salts should be limited to avoid the formation of a product of excessive water-solubility, as otherwise the laundry-resistance of the finished composition will be reduced. Thus, for example, about 5-7 mols of ethylene oxide should be condensed with mixtures in which the aliphatic radicals contain 16-18 carbon atoms, while quantities of 3-6 mols should be used with guanidines of lower molecular weight. Larger quantities of propylene or butylene oxides up to about 8-10 mols may be used, since the water-solubilizing action of these compounds is not as great as that of ethylene oxide. In general, therefore, about 2-10 mols of an alkylene oxide of 2-4 carbon atoms should be used in preparing the cationic softening agents employed in the softeners of our invention, the preferred compositions being those containing 5-7 mols of ethylene oxide for each mol of an aliphatic amine of 16-18 carbon atoms used as starting material.

Any anionic surface-active agent containing a single long aliphatic radical of 12 or more carbon atoms may be employed. Higher alkyl sulfates such as dodecyl, hexadecyl or octadecyl sulfate or alkaryl sulfonates such as keryl benzene sulfonate may be used if desired. However, we prefer to use the mono-esters or mono-amides of aliphatic sulfocarboxylic acids, since these have given good results in commercial practice. Mono-lauryl, monocetyl, monostearyl and monooleyl esters of sulfosuccinic acid, used as the disodium salts, have given very good results. Still better results are obtained with the corresponding sulfosuccinamates. These compounds have the formula:



in which R is a saturated or unsaturated aliphatic radical of 12 or more carbon atoms, and preferably an unbranched aliphatic chain of 16-18 carbon atoms and Me is a salt-forming group such as sodium, ammonium, etc. The hexadecyl and octadecyl sulfosuccinamates are preferred to the corresponding compounds of lower molecular weight because of their reduced water-solubility, and this is also true of the corresponding mono esters of sulfosuccinic acid.

One of the most important advantages of the compositions of our invention is the fact that they can be applied to textiles in conjunction with thermosetting resin finishes such as methylol melamines containing 3-6 methylol groups, di-

methylol urea, alkylated methylol melamines such as tri, tetra, penta or hexamethylated methylol melamines or with dimethylated dimethylol urea. These and similar resin finishes are usually applied from an aqueous bath which also contains an acidic or acid-releasing curing accelerator such as diammonium hydrogen phosphate, phthalic acid, oxalic acid and the like. Any of the softening compositions of our invention may be added to these baths in quantities suitable to

give the desired softness of hand in the finished textiles, since the stability of the bath is not reduced thereby. Moreover, we have found that the creaseproofing and shrinkproofing action obtained by the application of thermosetting resins is not impaired by the simultaneous application of our softening compositions. Textile finishing processes in which the softening compositions described above are applied in conjunction with resin finishes therefore constitute another

important feature of our invention.

The permanency of the softening agents of our invention is still further enhanced by the admixture of small quantities of water-soluble polyvalent metal salts therewith. However these quantities should be limited to not more than about 0.1-4%, based on the combined weight of the substituted carbamic acid salts and the anionic surface-active agent, since larger quantities of inorganic salts may cause harshness in the treated fabrics. In some cases the presence of substantial quantities of these inorganic salts may cause tendering of the treated fabrics, but this tendency can be overcome by the addition of small quantities of water-soluble amides such as urea, thiourea and the like. The presence of these quantities of polyvalent metal salts does not interfere with the application of the softening composition in conjunction with resins and resin finishes.

From the foregoing it will be seen that the improved textile softening compositions of our invention are those which contain a cationic softener consisting essentially of the condensation product of mixed aliphatic amine and aliphatic-substituted guanidine salts of N-aliphatic carbamic acids in which the aliphatic radicals contain 12-18 carbon atoms with 2-10 mols of an alkylene oxide of 2-4 carbon atoms, this cationic softener being mixed with an anionic surface-active agent containing a single long aliphatic radical of at least 12 carbon atoms. Preferably a substantial excess of the cationic softener is used, the preferred amounts being about 80-96% of the mixture. Cationic and anionic materials containing aliphatic radicals of 16-18 carbon

## 5

atoms are preferred, and in such mixtures optimum results are obtained with about 90-94% by weight of the cationic material and about 6-10% by weight of the anionic material. These compositions may be used as such or in admixture with 0.1-4% of water-soluble polyvalent metal salts such as aluminum sulfate, and in the latter case we prefer to add a water-soluble amide such as urea, thiourea and the like in amounts of about 1-5 times the weight of the metal salt.

The compositions of our invention may be applied to textiles by any of the known or approved methods for the application of softening agents. Thus, for example, they can be diluted with water to any desired consistency and textile materials, such as spun rayon, cotton or wool cloth may be impregnated with the resulting solutions. The cloth is then preferably heated for suitable times at temperatures of 200-400° F. to convert the softener into a water-insoluble condition, after which the finish possesses excellent laundry-resistance. This method of application may be combined with the application of other finishing agents such as resins, starch, etc., as will hereinafter be described in greater detail.

The invention will be further illustrated by the following specific examples, which describe the preparation of preferred ingredients and preferred softening compositions for textiles. It should be understood, however, that these examples are given primarily for purposes of illustration and that the invention in its broader aspects is not limited thereto.

## EXAMPLE 1

*Lauryl disodium sulfosuccinamate*

36 g. of primary laurylamine was added to 20 g. of maleic anhydride dissolved in 150 ml. of acetone at room temperature. The reaction mixture was then neutralized to a pH of 7.0 with a 45% solution of NaOH and the mixture evaporated to dryness to remove the acetone. The product was then stirred into a warm aqueous solution containing 50% alcohol and NaHSO<sub>3</sub>. After heating for two hours 90% of the theoretical quantity of NaHSO<sub>3</sub> had been consumed and the solution was again evaporated to dryness. The lauryl disodium sulfosuccinamate was then ground to a white powder easily soluble in water.

## EXAMPLE 2

*Tetradecyl disodium sulfosuccinamate*

Tetradecyl disodium sulfosuccinamate was prepared using the general procedure described in Example 1 employing a commercial grade (88.5%) of tetradecyl amine, C<sub>14</sub>H<sub>29</sub>NH<sub>2</sub>. The product was a white powder having a sweet odor and a bitter taste. It was fairly soluble in water, a 10% solution being slightly turbid at 30° C.

## EXAMPLE 3

*Octadecyl disodium sulfosuccinamate*

Octadecyl disodium sulfosuccinamate was prepared by the method described in Example 2 using commercial octadecyl amine, C<sub>18</sub>H<sub>37</sub>NH<sub>2</sub>. The product was a yellow waxy powder having a mildly soapy odor and taste. It was dispersed in water to a 35% paste.

## EXAMPLE 4

Mixtures of higher aliphatic-substituted guanidine salts with carbamates of the corresponding higher alkyl amines are prepared by reacting the

## 6

alkyl amines with aqueous cyanamide solutions in the presence of carbon dioxide. Reaction products in which about 15-40 mol percent of the amine has been converted into an aliphatic-substituted guanidine produce the best textile softening compositions. With less than 15% of the amine converted into guanidine the composition exhibits yellowing on the fabric, while with more than 40% the composition is too strongly basic and tends to neutralize acid curing agents of the type of diammonium hydrogen phosphate when used in textile finishing baths containing thermosetting resins.

A composition containing about 25-35% of the amine in the form of a higher aliphatic-substituted guanidine is formed by reacting the following materials:

|                                     | Parts by weight |
|-------------------------------------|-----------------|
| 20 Octadecylamine                   | 269             |
| Isopropyl alcohol                   | 135             |
| Carbon dioxide                      | 25              |
| Water                               | 17              |
| Cyanamide (23.9% solution in water) | 87.6            |

25 The amine is dissolved in the isopropyl alcohol by heating at 45° C. and then the solution is pumped into a reaction vessel along with the water. During 1.5 hours the carbon dioxide, in the form of dry ice, is added in small portions, the temperature being kept below 65° C. by cooling. The carbon dioxide reacts with the amine to form a salt.

The cyanamide solution is next added slowly over a period of about 4-5 hours under a reflux condenser, the reaction temperature being maintained at 83-89° C. Carbon dioxide gas is preferably bubbled through the reaction mixture during the addition of cyanamide to make sure that an excess is present at all times. After the cyanamide addition is complete the mixture is heated an additional hour.

40 Analysis of the composition prepared by this reaction has shown it to be a mixture of octadecylguanidinium-N octadecylcarbamate



and octadecyl amine N-octadecylcarbamate in which about 50% of the amine has been converted into N-octadecylcarbamate and about 30% is converted into mono octadecyl guanidine which is combined with a part of the octadecyl-substituted carbamic acid in the form of a guanidinium salt. The remainder of the amine is combined with the rest of the N-octadecyl carbamic acid in the form of a salt.

50 A considerably cheaper product of approximately the same molecular composition and having equally good softening properties is obtained by substituting commercial mixtures of higher aliphatic amines for the octadecyl amine in the above preparation. Thus, for example, a mixture containing about 25% of hexadecylamine, 25% of saturated octadecylamine and 50% of unsaturated primary amines of 18 carbon atoms is

65 available commercially in large quantities, and is a preferred raw material for the preparation of cationic softening compositions used in practicing the present invention. Corresponding mixtures of lower molecular weight but having the same molecular ratio of guanidine salt to N-aliphatic carbamate are obtained by the same procedure when laurylamine, myristylamine and other saturated and unsaturated aliphatic amines of 12-18 or more carbon atoms are substituted in the corresponding molecular quantities.

The guanidine carbamate mixture was condensed with alkylene oxide to form the condensation products used as cationic softeners in the compositions of the present invention. Upon completion of the procedure described above the vessel containing the reaction product was adapted for pressure and an ethylene oxide tank was attached so that ethylene oxide could be introduced above the surface of the reaction mixture. Ethylene oxide was slowly added at 60-66° C. at a rate such that the internal pressure did not exceed 20 lbs. per square inch. Sufficient ethylene oxide was added during about 4 hours so that the final product contained not less than 5 nor more than 7 mols of the oxide for each mol of amine used as starting material. This amounted to 220-308 parts by weight of ethylene oxide.

for use in a textile finishing bath having the following composition:

Component:

|                                   |               |      |
|-----------------------------------|---------------|------|
| Methylated methyol melamine (80%) | weight in lbs | 86.0 |
| Accelerator                       | do            | 2.4  |
| Softener                          | do            | 6.0  |
| Water to make                     | gallons       | 100  |

10 The accelerator was a mixture of approximately four parts by weight of hexamethylene tetramine and 30 parts of diammonium hydrogen phosphate.

Samples of rayon suiting were impregnated in this bath and squeezed to a 94% pickup. They were then cured 6 minutes at 290° F. and soaped five minutes, one-half hour, and one hour at 120° F. in 0.25% soap solution. Results on hand initially and after each laundering were as follows:

| After Cure                       | Softness as determined by hand |           |           |
|----------------------------------|--------------------------------|-----------|-----------|
|                                  | After soaping as follows:      |           |           |
|                                  | 5 min.                         | 30 min.   | 60 min.   |
| Softener A                       | Fair                           | Fair      | Fair      |
| Softener B                       | do                             | do        | do        |
| Softener C                       | do                             | Good      | Good      |
| Softener D                       | do                             | Fair      | Fair      |
| Softener E                       | Good                           | do        | Good      |
| Softener F                       | Very good                      | Good      | Good      |
| Softener G                       | do                             | Very good | Very good |
| Softener H                       | do                             | do        | do        |
| Commercial Softener <sup>1</sup> | do                             | do        | do        |
| Example 4 alone                  | do                             | Good      | Raggy     |
| Blank                            | do                             | Harsh     | Harsh     |

<sup>1</sup> Cetyl dimethyl benzyl ammonium chloride.

After the ethylene oxide addition was completed the product was heated to 90° C. for a few minutes, then cooled to 70° C. and allowed to stand overnight. The next day it was concentrated by evaporation under a partial vacuum until a 40 sample showed a solids content of 80% upon distillation with benzene. The concentrated product was a yellow syrup.

Other lower alkylene oxides such as propylene oxide or butylene oxide may be substituted for ethylene oxide in the above preparation but larger quantities up to 8-10 mols of these compounds may be used if desired. Reaction with alkylene oxides increases the water solubility of the aliphatic aminecyanamide-carbon dioxide reaction products and excessive quantities will form a product having too great a water solubility, which reduces the storage stability and laundry-resistance of the final textile finishing composition.

EXAMPLE 5

*Evaluation of softener compositions*

Various mixtures of the product of Example 4 with the product of Example 3 were prepared as shown in the following table:

| Softener         | A    | B    | C    | D    | E    | F    | G    | H    |
|------------------|------|------|------|------|------|------|------|------|
| Example 4 (100%) | 24.5 | 24.5 | 25.5 | 18.0 | 25.0 | 20.0 | 30.0 | 32.5 |
| Example 3 (35%)  | 38.0 | 38.0 | 20.0 | 37.5 | 24.0 | 30.0 | 12.5 | 6.5  |
| HCl              | 3.1  |      | 3.2  |      |      |      |      |      |
| Acetic Acid      |      | 1.8  |      |      |      |      |      |      |
| 2B Alcohol       | 15.5 | 24.5 | 25.5 |      |      |      |      |      |
| Water            | 18.9 | 11.2 | 26.8 | 44.5 | 51.0 | 50.0 | 57.5 | 61.0 |

In all cases the two surface-active agents were dissolved in separate portions of water at 120° F. and the solutions were mixed and stirred for 15 minutes or until homogeneous.

The mixtures were then evaluated as softeners

55 These results show that permanency against washing is obtained by mixing the cationic softeners with anionic surface-active agents throughout a range of ratios including as little as 58 parts by weight of the cationic softener to 42 parts by weight of the anionic surface-active agent (composition D) up to 93.5 parts of the softener to 6.5 parts of the anionic surface-active agent, as in composition H. However, the best

45 hands are obtained when the alkylene oxide condensation products are present in a substantial excess ranging from about 3-15:1. The cationic softeners alone will produce a very good hand on the resin-treated fabric, but are not resistant to soaping in the absence of the anionic surface-active agent.

EXAMPLE 6

55 The laundry-resistance of the finishes of the present invention is frequently increased by adding polyvalent metal salts which will insolubilize the anionic surface-active agent. This is particularly desirable when the softener is to be used alone; i. e., without resin or other binding agent of the type illustrated in the preceding example.

60 Although a wide variety of water-soluble polyvalent metal salts may be used, we prefer the water-soluble aluminum salts such as aluminum sulfate, since they do not discolor the goods.

65 The insolubilizing action of aluminum salts is shown by comparison of the following compositions:

|                                                                     | Composition of Softener |       |      |    |    |
|---------------------------------------------------------------------|-------------------------|-------|------|----|----|
|                                                                     | 1                       | 2     | 3    | 4  | 5  |
| Example 4 (80%)                                                     | 25                      | 25.00 | 25.0 | 25 | 25 |
| Example 3 (35%)                                                     | 5                       | 5.00  | 5.0  | 5  | 5  |
| Al <sub>2</sub> (SO <sub>4</sub> ) <sub>3</sub> ·18H <sub>2</sub> O | 0                       | 0.25  | 0.5  | 1  | 2  |
| Water                                                               | 70                      | 69.75 | 69.5 | 69 | 68 |

Pieces of blue spun rayon suiting were impregnated for one minute in 1% and 2% solutions of the above softeners, frame dried six minutes at 250° F., conditioned overnight and evaluated for softness of hand. They were then laundered several times and the hand after each laundering was determined. The results obtained are given in the following table:

| Softener | 5 min.          | 50 min.         | 1 hour          | 2 hours             |
|----------|-----------------|-----------------|-----------------|---------------------|
| 1.       | Very soft, full | Very soft, full | Very soft       | Soft but sl. raggy. |
| 2.       | do              | do              | Very soft, full | Full and soft.      |
| 3.       | do              | do              | do              | Do.                 |
| 4.       | Medium soft     | Medium soft     | Medium soft     | Do.                 |
| 5.       | Sl. harsh       | Sl. harsh       | Sl. harsh       | Sl. harsh.          |
| None     | Very harsh      | Harsh           | Harsh           | Harsh               |

The addition of a polyvalent metal salt such as aluminum sulfate in amounts of about 0.1-4% of the weight of the softener therefore assists materially in the retention of hand on soaping but the addition of too much of the metal salt causes harshness.

#### EXAMPLE 7

The following composition has been found to be an excellent softener for general use. It produces a soft hand on both proteic textiles such as silk, wool, nylon and vinyon and on cellulosic textiles such as cotton and spun rayon and may be applied alone or in conjunction with starch, thermosetting resins, or other types of finishes. It is usually applied in quantities of 0.1-5%, based on the dry weight of the textiles.

#### Per cent by weight

|                                                                     |       |
|---------------------------------------------------------------------|-------|
| Product of Example 4 (80% solids)                                   | 40    |
| Product of Example 3 (35% solids)                                   | 8     |
| Al <sub>2</sub> (SO <sub>4</sub> ) <sub>3</sub> .18H <sub>2</sub> O | 0.26  |
| Urea                                                                | 0.52  |
| Water                                                               | 51.22 |

The "product of Example 4" is preferably one in which the commercial mixture of hexadecyl and octadecylamines is used as a starting material.

This composition decreases the bleeding of dyed fabrics and does not cause dye fading, it does not chalk or dust upon storage of the treated textiles and it can be applied along with thermosetting resin finishes from the same bath without impairing the bath stability or the curing action of curing accelerators contained therein.

#### What we claim is:

1. A softening composition for textiles comprising a mixture of 90-94% by weight of the condensation product of 5-7 mols of ethylene oxide with a mixture of 50-70 mol percent of an aliphatic-substituted guanidinium N-aliphatic carbamate and 50-30 mol percent of an aliphatic amine N-aliphatic carbamate in which the aliphatic radicals contain 16-18 carbon atoms and 10-6% by weight of an anionic surface-active agent containing a single long aliphatic radical of 16-18 carbon atoms together with 0.1-4% of a water-soluble aluminum salt, based on the weight of said mixture.

2. A softening composition for textiles comprising a mixture of 90-94% by weight of the condensation product of 5-7 mols of ethylene oxide with a mixture of 50-70 mol percent of an aliphatic-substituted guanidinium N-aliphatic carbamate and 50-30 mol percent of an aliphatic amine N-aliphatic carbamate in which the aliphatic radicals contain 16-18 carbon atoms and

10-6% by weight of an anionic surface-active agent of the formula



in which Me is a monovalent salt-forming radical and X is a member of the group consisting of —OR and —NHR, R being an aliphatic radical

5

20

25

30

35

40

45

50

55

60

65

70

75

80

85

90

95

100

of 12-18 carbon atoms, together with 0.1-4% of a water-soluble aluminum salt, based on the weight of said mixture.

3. A softening composition for textiles comprising a mixture of 90-94% by weight of the condensation product of 5-7 mols of ethylene oxide with a mixture of 50-70 mol percent of an aliphatic-substituted guanidinium N-aliphatic carbamate and 50-30 mol percent of an aliphatic amine N-aliphatic carbamate in which the aliphatic radicals contain 16-18 carbon atoms and 10-6% by weight of an N-aliphatic disodium sulfosuccinamate in which the aliphatic radical contains 16-18 carbon atoms, together with 0.1-4% of aluminum sulfate, based on the weight of said mixture, and urea in amounts about twice the weight of said aluminum sulfate.

4. A softening composition for textiles comprising 58 to 96 parts by weight of the condensation product of a mixture of aliphatic amine and aliphatic-substituted guanidine salts of N-aliphatic carbamic acids in which the aliphatic radicals contain 12 to 18 carbon atoms with 2 to 10 mols of an alkylene oxide of 2 to 4 carbon atoms and 42 to 4 parts by weight of an anionic surface-active agent containing a single long aliphatic radical of 12 to 18 carbon atoms.

5. A composition according to claim 4 in which the mixture of aliphatic amine and aliphatic-substituted guanidine salts of N-aliphatic carbamic acids is condensed with 3 to 7 mols of ethylene oxide.

6. A composition according to claim 5 in which the anionic surface-active agent is a compound of the formula



in which Me is a monovalent salt-forming radical and X is a member of the group consisting of —OR and —NHR, R being an aliphatic radical of 12-18 carbon atoms.

7. A composition according to claim 6 which also contains 0.1 to 4% of a water-soluble polyvalent metal salt, based on the weight of the mixture recited in claim 6.

8. A composition according to claim 7 which also contains a water-soluble amide in an amount of about 1 to 5 times the weight of said polyvalent metal salt.

9. A composition according to claim 4 in which a mixture of aliphatic amine and aliphatic-substituted guanidine salts of N-aliphatic carbamic acids in which the aliphatic radicals contain 16-18 carbon atoms is condensed with 5-7 mols of ethylene oxide.

10. A softening composition for textiles comprising 58 to 96 parts by weight of the condensa-

tion product of a mixture of 50-70 mol per cent of an aliphatic-substituted-guanidinium N-aliphatic carbamate and 50-30 mol per cent of an aliphatic amine N-aliphatic carbamate in which the aliphatic radicals contain 12-18 carbon atoms with 2-10 mols of an alkylene oxide of 2-4 carbon atoms and 42 to 4 parts by weight of an anionic surface-active agent containing a single long aliphatic radical of 12 to 18 carbon atoms.

11. A composition according to claim 10 in which the mixture of aliphatic amine and aliphatic-substituted guanidine salts of N-aliphatic carbamic acids is condensed with 3 to 7 mols of ethylene oxide.

12. A composition according to claim 11 in which the anionic surface-active agent is a compound of the formula



in which Me is a monovalent salt-forming radical and X is a member of the group consisting of —OR and —NHR, R being an aliphatic radical of 12-18 carbon atoms.

13. A composition according to claim 12 which also contains 0.1 to 4% of a water-soluble polyvalent metal salt, based on the weight of the mixture recited in claim 12.

14. A composition according to claim 13 which also contains a water-soluble amide in an amount of about 1 to 5 times the weight of said polyvalent metal salt.

15. A composition according to claim 10 in which a mixture of aliphatic amine and aliphatic-substituted guanidine salts of N-aliphatic carbamic acids in which the aliphatic radicals contain 16-18 carbon atoms is condensed with 5-7 mols of ethylene oxide.

16. A softening composition for textiles comprising 80-96% by weight of the condensation product of a mixture of aliphatic amine and aliphatic-substituted guanidine salts of N-aliphatic carbamic acids in which the aliphatic radicals contain 12-18 carbon atoms with 2-10 mols of an alkylene oxide of 2-4 carbon atoms and 20-4% by weight of an anionic surface-active agent containing a single aliphatic radical of 12-18 carbon atoms.

17. A composition according to claim 16 in which the mixture of aliphatic amine and aliphatic-substituted guanidine salts of N-aliphatic carbamic acids is condensed with 3 to 7 mols of ethylene oxide.

18. A composition according to claim 17 which also contains 0.1 to 4% of a water-soluble polyvalent metal salt based on the weight of the mixture recited in claim 6.

19. A composition according to claim 18 which also contains a water-soluble amide in an amount of about 1 to 5 times the weight of said polyvalent metal salt.

EMIL A. VITALIS.  
JOHN E. LYNN.

#### REFERENCES CITED

The following references are of record in the file of this patent:

#### UNITED STATES PATENTS

| Number       | Name      | Date          |
|--------------|-----------|---------------|
| 2,258,321    | Ericks    | Oct. 7, 1941  |
| 2,299,012    | Ericks    | Oct. 13, 1942 |
| 35 2,142,688 | Brodersen | Jan. 3, 1939  |
| 2,304,113    | Morgan    | Dec. 8, 1942  |
| 2,236,074    | Schwartz  | Mar. 25, 1941 |
| 2,252,401    | Jaeger    | Aug. 12, 1941 |